

## 1

3,399,027

**DYEING NICKEL CHELATE MODIFIED POLY-OLEFIN WITH AZOMETHINE DYES**

Gérald Siegrist, Riehen, and Walter Biedermann, Basel, Switzerland, assignors to J. R. Geigy A.G., Basel, Switzerland

No Drawing. Filed Aug. 15, 1963, Ser. No. 302,465  
Claims priority, application Switzerland, Aug. 20, 1962,  
9,930/62

4 Claims. (Cl. 8—31)

**ABSTRACT OF THE DISCLOSURE**

Shaped polyolefines which contain organic nickel chelate complexes as dye acceptors are dyed or printed by contacting shaped articles of such polyolefine material with fine dispersions, either in the form of solution or fine suspensions of certain metallizable azo or azomethine dyestuffs which are capable of taking part in metal complex formation.

The present invention concerns a process for the dyeing and printing of shaped goods made from polyolefines and more particularly from polypropylene or polyethylene material, as well as an industrial product, the shaped polyolefine goods colored or printed according to this process.

To the best of our knowledge, no fully satisfactory dyeing process for previously shaped polyolefine articles, in particular polyethylene and polypropylene fibers was hitherto known; up to the present, dyeings attained by subjecting such previously formed material to a dyeing or printing process were of weak color depth and only of mediocre fastness to light.

It is, therefore, an object of our invention to provide shaped, colored olefine, and particularly polypropylene or polyethylene articles of deep shades and good fastness to light.

It has now surprisingly been found that shaped articles of polyolefine material of strong and light-fast shades are obtained by dyeing or printing such articles, the polyolefine of which contains organic nickel chelate complexes as dye acceptors, with fine dispersions, either in the form of solutions or fine suspensions of certain metallizable azo or azomethine dyestuffs defined below which are free from salt-forming, water-solubilizing groups, or containing only such salt-forming groups as defined below, which are capable of taking part in metal complex formation.

It is thus possible to attain the above-stated object as well as others that will become apparent as the description of the invention proceeds. The resulting dyed and printed polyolefine goods are distinguished particularly by a light-fastness which is due, on the other hand to the good light-fastness properties of the resulting dye component in the colored material and, on the other hand, to the fact that the organic nickel chelate complexes have the double function of acting as dye acceptors and as light stabilizers, the combined effect being an excellent light-fastness of the dyed polyolefine article.

The term "organic nickel chelate complexes" is used herein to describe polydentate organic chelating agents capable of acting as dye acceptors which preferably contain several oxygen atoms and in certain cases, in addition, sulfur or nitrogen atoms as donor atoms.

The starting polyolefine material which is dyed according to the invention contains preferably nickel chelate complexes of the aromatic series, preferably of alkylated o,o'-dihydroxydiphenyl sulfides, each of the alkyl radicals advantageously containing about 4 to 12 carbon atoms. Polyolefine, which contains the nickel complex of 2,2'-dihydroxy-5,5'-diisooctylidiphenyl sulfide is particularly suitable for the dyeing process according to the invention.

## 2

tion because remarkable deep dyeings can be attained therewith. Other polyolefines containing a nickel chelate complex which are suitable for use according to the invention, are those containing nickel acetylacetone, nickel glycinate, 8-hydroxy-quinoline nickel complex, o-dihydroxy-benzene nickel complex, o-hydroxy benzophenone nickel complex, salicylaldehyde nickel complex radicals; Ni-ethylene diamine tetraacetate can be used as second choice only, with less improvement in fastness of the dyeings. The foregoing other chelate complexes are preferred.

Primarily, polypropylene e.g. isotactic polypropylene, is used as polyolefine but also polyethylene as well as mixed polymers of these two olefines containing the above-defined nickel chelates, can be dyed or printed according to the invention.

In addition to the nickel chelate complexes as defined, these polyolefines advantageously contain other additives such as antioxidants, additional light stabilizers, delustering agents, etc. The polyolefine material can be used in any form desired, e.g. as foils, granulates, and the like disperse dyes, but, preferably, as fibers. Advantageously, the content of nickel is about 0.1 to not more than 2% and preferably 0.1 to 1.2% of the weight of the material to be dyed; lower contents than 0.1% have a disadvantageous effect on the fastness properties of the resulting dyeings or prints.

The following classes of azo and azomethine dyestuffs are suitable for the dyeing and printing of the above-described polyolefine materials in the process according to the invention.

(1) Monoazo dyestuffs of the benzene-azobenzene and the benzene-azo-naphthalene series wherein one benzene nucleus must be substituted in o-position to the azo bridge by a hydroxy or —COOH group, while the other benzene nucleus or the naphthalene nucleus is substituted in o-position to the azo bridge by a —OH, —NH<sub>2</sub> or —NHR group, wherein R is either lower alkyl, phenyl, lower alkyl-phenyl, chlorophenyl, bromophenyl or ortho-carboxyphenyl.

(2) Disazo dyestuffs which are derived from the dyestuffs defined above under (1), wherein one benzene ring bears, in p-position to the azo bridge or in p-position to a metallizable hydroxy substituent defined above, a benzene-azo or naphthalene-azo substituent.

These dyestuffs defined above under (1) and (2) either bear no further substituents, or they are further ring-substituted, preferably in a position other than ortho, to the metallizable azo bridge, namely, alkyl with from 1 to preferably not more than 12 carbon atoms, e.g. methyl, ethyl, propyl, butyl, amyl, hexyl, octyl, decyl or dodecyl; cyclo-aliphatic substituents, particularly cyclohexyl; araliphatic substituents, particularly benzyl or phenylethyl; aromatic substituents, especially phenyl, chlorophenyl, bromophenyl, lower alkyl-phenyl, lower alkoxy-phenyl, nitrophenyl; lower alkoxy, e.g. ethoxy or methoxy; cyclo-alkoxy, particularly cyclohexyloxy; aralkoxy, especially benzyloxy; aryloxy, especially phenoxy or lower alkoxy-phenoxy; acylamino substituents, especially alkanoyl-amino, preferably with a total of from 2 to 7 carbon atoms; halogen substituents such as fluorine, chlorine or bromine; carbamyl or sulfamyl groups wherein the nitrogen atom is mono-substituted with alkyl with 1 to 8 carbon atoms, or phenyl, or cyclohexyl, or wherein the nitrogen atom is di-substituted with two alkyl groups or with one alkyl and one phenyl or one alkyl and one alkyl-phenyl radical, the total number of carbon atoms of the two nitrogen substituents being from 2 to 8; sulfonic acid aryl ester radicals, especially phenoxy sulfonyl, alkyl sulfonyl with from 1 to 6, and preferably from 3 to 6 carbon atoms, phenylsulfonyl, lower alkyl phenylsulfonyl, lower alkoxy carbonyl, lower alkoxy carbonyl amino, alkoxy

60 atoms; phenylsulfonyl, lower alkyl phenylsulfonyl, lower alkoxy carbonyl, lower alkoxy carbonyl amino, alkoxy

carbonyl with a total of from 2 to 8 carbon atoms, cyano, trifluoromethyl, amino, hydroxyl and/or nitro substituents.

The term "lower" as used herein in connection with an aliphatic group means that the group has from 1 to not more than 4 carbon atoms.

(3) Monoazo dyestuffs of the benzene-azo-pyrazol-5-one and the benzene-azo-(5-amino-pyrazole) series, wherein in the 1-position of the pyrazole nucleus is substituted with lower alkyl, phenyl, or naphthyl and the 3-position is substituted with lower alkyl or carbamyl, or carbamyl wherein in the nitrogen atom is either mono-substituted with alkyl with 1 to 8 carbon atoms or phenyl, or cyclohexyl, or wherein in the nitrogen atom is di-substituted with two alkyl groups or with one alkyl and one phenyl or one alkyl and one alkyl-phenyl radical, the total number of carbon atoms of the two nitrogen substituents being from 2 to 8, wherein in the benzene ring bears, in o-position to the azo bridge, one of the substituents —OH and —COOH. The remaining positions of the benzene ring are either unsubstituted or substituted by the ring substituents listed above for (1) and (2).

(4) Disazo dyestuffs derived from the monoazo dyestuffs described under (3), wherein the benzene ring is substituted in p-position to the azo bridge or in p-position to the metallizable —OH substituent with phenylazo or naphthylazo.

Again, the benzene or naphthalene nuclei of the dyestuff molecules defined under (3) and (4) are either free from further substituents or contain substituents from the class defined above as permissible ring substituents.

(5) Monoazo dyestuffs of the naphthalene-azo-benzene or the naphthalene-azo-naphthalene series, wherein one naphthalene nucleus bears, in o-position to the azo bridge, a metallizable —COOH group, while the other component, either a benzene or a naphthalene ring, bears in o-position to the azo bridge a —OH, —NH<sub>2</sub> or —NHR group, wherein R is either lower alkyl, phenyl, lower alkyl-phenyl, chlorophenyl, bromophenyl or ortho-carboxyphenyl.

(6) Monoazo dyestuffs of the naphthalene-azo-pyrazol-5-one and the naphthalene-azo-(5-amino-pyrazole) series, wherein the naphthalene nucleus bears, in o-position to the azo bridge, a —COOH group. The naphthalene, and especially benzene, nuclei of these dyestuffs where the latter are present in 1-position at the pyrazole nucleus are either unsubstituted or substituted with ring substituents of the class defined above; the pyrazole nuclei are substituted in 1- and 3-position as defined under (3).

(7) Azomethine dyestuffs of the benzene-azo-methine-benzene and the benzene-azo-benzene-naphthalene series, wherein the benzene nucleus linked to the nitrogen atom of the azomethine bridge bears, in o-position to said bridge, a —OH or —COOH group while the nucleus of the other component bears, in o-position to the bridge, a hydroxy group. The nuclei of these dyestuffs are either free from further substituents or bear further ring-substituents of the class defined above.

(8) Azomethine dyestuffs derived from the dyestuffs defined in (7) above, wherein either the benzene ring linked to the nitrogen atom of the azomethine bridge bears, in p-position to said bridge or in p-position to a metallizable —OH group, or wherein a benzene nucleus linked to the methine group of the azomethine bridge bears, in p-position to the metallizable hydroxy group, a phenylazo or naphthylazo substituent. The aromatic nuclei of these dyestuffs are either free from further substituents or are further substituted with ring-substituents of the class defined above.

(9) Azomethine dyestuffs of the naphthalene-azo-methine-benzene or the naphthalene-azo-methine-naphthalene series, wherein the naphthalene nucleus linked to the nitrogen atom of the azomethine bridge bears, in o-position to said bridge, a —COOH group, while the nucleus of the other component bears, in o-position to said bridge, a hydroxyl group. The aryl nuclei of these

dyestuffs are either unsubstituted or substituted with ring-substituents of the class described above.

Primarily the metallizable groups in the o,o'-positions of azo or azomethine compounds are responsible for the metallization of these dyestuffs, e.g. hydroxyl, carboxyl or amino groups. However, other dyestuffs with a different type of metal complexing configuration which contain an o(lower alkyl - carbonyl)phenol - hydroxy-carboxy-hydroxy-phenyl-o-amino-carboxyphenyl grouping such as the o-acetyl-phenol or salicylic acid radical, can also be used. Of this last-mentioned group of dyestuffs, there are used especially

(10) The monoazo dyestuffs of the benzene-azo-3-carboxy-4-hydroxy-benzene series and the benzene-azo-3-carboxy-4-amino-benzene series and the disazo dyestuffs of the benzene-azo-benzene-azo-3-carboxy-4-hydroxy-benzene series. The benzene nuclei of these dyestuffs are either unsubstituted or substituted with ring-substituents of the class described above.

Substituents of a hydrophobic character, in particular alkyl radicals having 4 to 12 carbon atoms, but also the nitro group and/or halogen substituents, especially chlorine, bromine or fluorine, or trifluoromethyl, are preferred ring-substituents. When orange, brown, olive, bordeaux or gray shades are to be produced, particularly good results are obtained with the dyestuffs defined above under (1), (2), (3) and (4), the phenyl-azo substituent being preferred in the case of dyestuffs defined under (2) and (4), in which preferred classes of dyestuffs the carbocyclic nuclei are either free from further ring-substituents or substituted with alkyl having 4 to 12 carbon atoms, fluorine, chlorine, bromine and/or nitro.

When yellow shades are to be obtained, azomethine dyestuffs defined above under (7) and (8) are preferred, in which the aromatic nuclei are either unsubstituted or substituted with alkyl having 4 to 12 carbon atoms, nitro, fluorine, chlorine or bromine.

Dyeing is performed from a weakly alkaline, neutral or weakly acid, preferably aqueous dyebath wherein the dyestuff is finely dispersed as a solution and/or a fine suspension, preferably at boiling temperature, or at a temperature above 100° C. under corresponding excess pressure. Aqueous dispersions used as the dyebath according to the invention preferably contain as dispersing agents condensation products of formaldehyde and naphthalene sulfonic acids, of unsulfonated or sulfonated amines and higher fatty acids, e.g., of p-anisidine sulfonic acid with coconut oil fatty acid in a molar ratio of 1:1 or polyethylene-glycol ether of fatty alcohols with ethylene oxide in a molar ratio of from 1:10 to 1:20. Contact time between the dyebath and the goods to be dyed is preferably about 30 to 120 minutes.

It is particularly surprising that, in this relatively short time, there occurs formation of nickel dyestuff complexes by a metathetic reaction with at least a substantial portion (ca. 5%) to all of the organic nickel chelate dye acceptors initially present in the polyolefine material being dyed.

Printing is performed with a printing paste which contains the usual thickeners, e.g. water-soluble salts of alginic acids or crystal gum solution as well as, optionally, other additives usual in textile printing, such as urea. After printing, the print is fixed by known methods, e.g. by steaming at higher temperatures, preferably not exceeding about 145° C. in the case of polypropylene and not exceeding 115° C. in the case of polyethylene.

The dyeings and prints on polyolefine articles, in particular of polypropylene fibers produced by the process according to the invention, are very strong in color, and they also have good wet and wash fastness including fastness to perspiration, as well as fastness to light, to rubbing, to sublimation, to migration and to gas fumes.

These outstanding fastness properties are due to the formation, particularly in the surface strata of the polyolefine material, of chelate complexes of the nickel atoms

derived from the chelate dye complex-forming radicals of the metallizable dyestuff, acceptor molecules present therein, with at least a substantial portion of the aforesaid chelate complexes, formed at least during a dyeing treatment of about 30 to 60 minutes, consisting of complexes of the formula



wherein A is a dye acceptor radical selected from the group consisting of alkylated diphenyl sulfide nickel chelate, nickel acetylacetone, Ni-salt of glycine, 8-hydroxy-quinoline nickel complex, o-dihydroxy-benzene nickel complex, o-hydroxy-benzophenone nickel complex, salicylic aldehyde nickel complex radicals, and

B represents the radical of one of the dyestuffs defined above under (1) to (10),

$X_1$  and  $X_2$  being the residues of two metallizable substituents as defined supra.

All dyestuffs of classes (1) to (10) must be free from  $-\text{SO}_3\text{H}$  substituents and also from such  $-\text{COOH}$  and the like salt-forming substituents unless the latter are capable of chelating nickel atoms present in the polyolefine material being dyed.

The following examples illustrate the invention. Where not otherwise stated, parts and percentages are given by weight. The temperatures are in degrees centigrade. The relationship of parts by weight to parts by volume is as that of grams to cubic centimeters.

#### Example 1

(a) 250 parts of unstabilized polypropylene powder, 0.25 part of 2,2'-dihydroxy-3,3'-di-tert. butyl-5,5'-diethyl-diphenylmethane and 3.75 parts of the complex nickel compound from 1 atom of nickel and 2 molecules of 2,2'

35 25 dihydroxy-5,5'-di-tert. octyl-diphenyl sulfide are mixed together in a dry state, then homogenized on a set of mixing rollers at 180° for 5 to 10 minutes and finally sheeted into a foil of 0.5 mm. thickness.

Strips of 6 x 50 mm. of cuts from this foil and 6 to 8 parts thereof are fed into the cylinder of a melt index tester of the type described in the "Tentative Method of Test for Measuring Flow Rates of Thermoplastics by Extrusion Plastometer," ASTM Designation: D1238-57T, issued 1952; revised 1957.

As soon as the temperature of the cylinder has attained 230-250°, the polypropylene is extruded and simultaneously wound onto a perforated drum. The monofilament so obtained is stretched at the ratio of from 1:6 to 1:8 by rewinding over a stretching device operating at room temperature.

(b) 100 parts of the fibers produced according to the above instructions are treated in a dyebath consisting of 5000 parts of water, 2.5 parts of sodium N-oleyl-N-methyl-aminoethylsulfonate, 2.5 parts of ammonium sulfate and 2 parts of a dyestuff preparation produced by milling 3 parts of the monoazo dyestuff of the formula



with 4 parts of the disodium salt of dinaphthylmethane disulfonic acid. The fabric is introduced into the 50° warm bath, the temperature is raised to the boil within 30 minutes and the bath is kept at this temperature for 60 minutes. The fabric is then rinsed hot and cold.

An orange colored fiber is obtained which is fast in particular to light, washing and rubbing.

#### Example 2

10 Example 1 is reacted, but 3.75 parts of nickel acetylacetone are used instead of 3.75 parts of the complex nickel compound from 1 atom of nickel and 2 molecules of 2,2'-dihydroxy-5,5'-di-tert. octyl-diphenyl sulfide; colored fibers are obtained which are also dyed on orange shade with the dyestuff mentioned in Example 1. The dyeings are also fast to light and washing.

#### Example 3

20 Example 1 is repeated, but instead of the dyestuff used in the same process, 2 parts of a dyestuff preparation from 3 parts of the monoazo dyestuff of the formula



25 and 4 parts of the disodium salt of dinaphthylmethane disulfonic acid are used; a dark violet-colored fiber is obtained which has good fastness, among others, to light, washing and rubbing.

#### Example 4

30 35 100 parts of yarn produced according to part (a) of Example 1 treated in a dyebath obtained from 5000 parts of water, 2.5 parts of ammonium sulfate and 2 parts of a dyestuff preparation produced by milling 3 parts of the dyestuff of the formula



45 45 with 4 parts of the disodium salt of dinaphthylmethane disulfonic acid. The fabric is introduced into 50° warm bath, the temperature is raised to the boil within 30 minutes and the bath is kept at this temperature for 60 minutes. The fabric is then rinsed hot and cold.

50 Yellow-colored fibers are obtained which are fast especially to light, washing and rubbing.

#### Example 5

55 Example 4 is repeated, but instead of the dyestuff used therein, 2 parts of a dyestuff preparation from 3 parts of the monoazo dyestuff of the formula



60 65 and 4 parts of the disodium salt of dinaphthylmethane disulfonic acid are used; a bordeaux colored fiber which has good fastness particularly to light, washing and rubbing is obtained.

#### Example 6

70 75 A fabric made from the nickel-containing polypropylene fibers produced by the process described in part (a)

of Example 1 is dyed with 2 parts of the dyestuff preparation from 3 parts of the monoazo dyestuff of the formula



10

and 4 parts of the disodium salt of dinaphthylmethane disulfonic acid, under the conditions and with the other ingredients described in Example 4. An orange colored material which has good fastness especially to light, washing and rubbing is obtained.

#### Example 7

A fabric made from the nickel-containing polypropylene fibers produced by the process described is dyed with 2 parts of the dyestuff preparation from 3 parts of the disazo dyestuff of the formula



and 4 parts of the disodium salt of dinaphthylmethane disulfonic acid, according to the method described in Example 1, all other ingredients and conditions remaining unchanged. A blueish brown colored material is obtained which has good fastness, among others, to light, washing and rubbing.

#### Example 8

100 parts of yarn, produced according to part (a) of Example 1, in the form of cheese are dyed in a closed circulation apparatus in a dyebath consisting of 2000 parts of water which has been made alkaline (pH about 9) with trisodium phosphate, 2 parts of the condensation product of p-anisidine sulfonic acid and coconut oil fatty acid, molar ratio 1:1, and 2 parts of a dyestuff of the formula



The goods are entered at 50°, the bath is brought to 110° within 30 minutes, the goods are dyed for 30 minutes at this temperature and then rinsed first hot and then cold.

A vivid yellow-colored yarn is obtained which has good fastness especially to light, washing and rubbing.

#### Example 9

Example 8 is repeated, but instead of the dyestuff there mentioned, 2 parts of the dyestuff of the formula



are used; an orange-colored yarn is obtained which has good fastness to in particular light, washing and rubbing.

#### Example 10

A fabric made from nickel-containing polypropylene fiber produced as described in paragraph (a) of Example 1, is printed with a printing paste of the following composition: 20 g. of the dyestuff preparation from 8.6 parts of the monoazo dyestuff of the formula



15

|                           | G.    |
|---------------------------|-------|
| Urea                      | 40    |
| Water                     | 340   |
| Crystal gum solution, 25% | 600   |
|                           | 1,000 |

The print is dried, steamed for 30 minutes at an excess pressure of 0.5 atmosphere and then rinsed first with hot and then with cold water.

25 A fabric printed a reddish brown color is obtained. The dyeing has good fastness especially to light, washing and rubbing.

#### Example 11

In the printing paste of Example 10, which is repeated 30 with otherwise the same procedure, there are used, instead of the dyestuff given therein, 20 g. of a dyestuff preparation from 8.6 parts of the monoazo dyestuff of the formula



35

and 11.4 parts of the disodium salt of dinaphthylmethane disulfonic acid; gray prints are obtained on the fabric of nickel-containing polypropylene fibers, which prints are fast especially to light, washing and rubbing.

#### Example 12

50 250 parts of low-pressure polyethylene granulate containing 0.25 parts of tert. butyl-p-cresol and 0.75 part of dilauryl thiodipropionate as stabilizers, are thoroughly mixed in a mixing drum with 3.75 parts of finely pulverized nickel acetylacetone. The granules are then melted in an extruder and a monofilament is extruded at a temperature of 180° through a die of 1.0 mm. diameter. The monofilament obtained is stretched on a hot apparatus to 55 six times its length.

100 parts of the fiber produced as described above are treated in a dyebath consisting of 5000 parts of water, 2.5 parts of sodium N-oleyl-N-methyl-amino - ethylsulfonate, and 2.5 parts of ammonium sulfate and 2 parts of dyestuff preparation produced by milling 3 parts of the monoazo dyestuff of the formula



65 with 4 parts of the disodium salt of dinaphthyl methane disulfonic acid.

The monofilament is entered at 50° into the dye-bath, the temperature is raised to 90° within 30 minutes and the bath is kept at this temperature for 60 minutes.

A deep grey-colored monofilament is obtained. The dyeing is fast to light, washing and rubbing.

By using with otherwise the same procedure for the production of the polyethylene monofilament, 3.75 parts of the complex nickel compound obtained from one atom of nickel and 2 molecules of 2,2'-dihydroxy-5,5'-di-tert. octyl diphenyl sulfide instead of the 3.75 parts of nickel acetyl acetonate, there is obtained with the same dyestuff a filament which is also dyed deep grey, and has similar good fastness properties.

We claim:

1. A process for coloring shaped goods of a polyolefine material selected from the group consisting of shapable polyethylene and shapable polypropylene, comprising, in combination:

(a) admixing with said polyolefine an organic nickel chelate selected from the group consisting of alkylated O,O'-dihydroxydiphenyl sulfide nickel chelate, nickel acetylacetone, Ni-salt of glycine, 8-hydroxy-quinoline nickel complex, o-dihydroxy-benzene nickel complex, o-hydroxybenzophenone nickel complex, salicylic aldehyde nickel complex and ethylene diamine tetraacetate in an amount corresponding to from about 0.1 to 1.2% by weight of nickel in the resulting nickel chelate-containing polyolefine material, and shaping the polyolefine, and

(b) contacting the resulting shaped nickel chelate-containing polyolefine goods with an aqueous dispersion of an azomethine dyestuff selected from the group consisting of a benzene-N=CH-benzene dyestuff and a benzene-N=CH-naphthalene dyestuff, wherein the benzene nucleus linked to the nitrogen atom of the azomethine bridge bears, in o-position to said bridge, a metallizable substituent selected from the group consisting of —OH and —COOH, and the nucleus of the other dyestuff moiety bears a metallizable —OH group in o-position to said bridge, said azomethine dyestuff being free from —SO<sub>3</sub>H groups and non-chelatable —COOH groups, for at least about 30 minutes at a temperature ranging from about 100° C. to a temperature not exceeding 115° C. in the case of polyethylene and about 145° C. in the case of polypropylene, the molar ratio to the nickel chelate present in the polyolefine goods being colored not exceeding substantially 1:1.

2. A process for coloring shaped goods of a polyolefine material selected from the group consisting of shapable polyethylene and shapable polypropylene, comprising, in combination:

(a) admixing with said polyolefine an organic nickel chelate selected from the group consisting of alkylated O,O'-dihydroxydiphenyl sulfide nickel chelate, nickel acetylacetone, Ni-salt of glycine, 8-hydroxy-quinoline nickel complex, o-dihydroxy-benzene nickel complex, o-hydroxybenzophenone nickel complex, salicylic aldehyde nickel complex and ethylene diamine tetraacetate in an amount corresponding to from about 0.1 to 1.2% by weight of nickel in the resulting nickel chelate-containing polyolefine material, and shaping the polyolefine, and

(b) contacting the resulting shaped nickel chelate-containing polyolefine goods with an aqueous dispersion of a dyestuff consisting of the monovalent radical of a monoazo dyestuff selected from the group consisting of a benzene-N=CH-benzene dyestuff and a benzene-N=CH-naphthalene dyestuff, wherein the benzene nucleus linked to the nitrogen atoms of the azomethine bridge bears, in o-position to said bridge, a metallizable —OH group, and the nucleus of the other dyestuff moiety bears a metallizable —OH group in o-position to said bridge, and wherein the benzene ring linked to the nitrogen atom of the azomethine bridge bears in one of the positions: para to said bridge and para to a metallizable —OH group, a substituent selected from the group consisting of phenyl-N=N- and naphthyl-N=N-, said dyestuff being free from —SO<sub>3</sub>H groups and non-chelatable

5

10

10

—COOH groups, for at least about 30 minutes at a temperature ranging from about 100° C. to a temperature not exceeding 115° C. in the case of polyethylene and about 145° C. in the case of polypropylene, the molar ratio to the nickel chelate present in the polyolefine goods being colored not exceeding substantially 1:1.

3. A process for coloring shaped goods of a polyolefine material selected from the group consisting of shapable polyethylene and shapable polypropylene, comprising, in combination:

(a) admixing with said polyolefine an organic nickel chelate selected from the group consisting of alkylated O,O'-dihydroxydiphenyl sulfide nickel chelate, nickel acetylacetone, Ni-salt of glycine, 8-hydroxy-quinoline nickel complex, o-dihydroxy-benzene nickel complex, o-hydroxybenzophenone nickel complex, salicylic aldehyde nickel complex and ethylene diamine tetraacetate in an amount corresponding to from about 0.1 to 1.2% by weight of nickel in the resulting nickel chelate-containing polyolefine material, and shaping the polyolefine, and

(b) contacting the resulting shaped nickel chelate-containing polyolefine goods with an aqueous dispersion of a dyestuff consisting of the monovalent radical of a benzene-N=CH-benzene dyestuff wherein the benzene nucleus linked to the nitrogen atom of the azomethine bridge bears, in o-position to said bridge, a metallizable substituent selected from the group consisting of —OH and —COOH, and the nucleus of the other dyestuff moiety bears a metallizable —OH group in o-position to said bridge, and wherein the latter nucleus bears, in para-position to said metallizable —OH group, a substituent selected from the group consisting of phenyl-N=N- and naphthyl-N=N-, said dyestuff being free from —SO<sub>3</sub>H groups and non-chelatable —COOH groups, for at least about 30 minutes at a temperature ranging from about 100° C. to a temperature not exceeding 115° C. in the case of polyethylene and about 145° C. in the case of polypropylene, the molar ratio to the nickel chelate present in the polyolefine goods being colored not exceeding substantially 1:1.

4. A process for coloring shaped goods of a polyolefine material selected from the group consisting of shapable polyethylene and shapable polypropylene, comprising, in combination:

(a) admixing with said polyolefine an organic nickel chelate selected from the group consisting of alkylated O,O'-dihydroxydiphenyl sulfide nickel chelate, nickel acetylacetone, Ni-salt of glycine, 8-hydroxy-quinoline nickel complex, o-dihydroxy-benzene nickel complex, o-hydroxybenzophenone nickel complex, salicylic aldehyde nickel complex and ethylene diamine tetraacetate in an amount corresponding to from about 0.1 to 1.2% by weight of nickel in the resulting nickel chelate-containing polyolefine material, and shaping the polyolefine, and

(b) contacting the resulting shaped nickel chelate-containing polyolefine goods with an aqueous dispersion of an azomethine dyestuff which is a member selected from the group consisting of a naphthalene-N=CH-benzene dyestuff and a naphthalene-N=CH-naphthalene dyestuff, wherein the naphthalene nucleus linked to the nitrogen atom of the azomethine bridge bears, in o-position to said bridge, a metallizable —COOH group, and the nucleus of the other dyestuff moiety bears a metallizable —OH group in o-position to said bridge, said azomethine dyestuff being free from —SO<sub>3</sub>H groups and non-chelatable —COOH groups, for at least about 30 minutes at a temperature ranging from about 100° C. to a temperature not exceeding 115° C. in the case of polyethylene and about 145° C. in the case of polypropylene, the molar ratio

70

75

11

to the nickel chelate present in the polyolefine goods  
being colored not exceeding substantially 1:1.

12

|           |        |               |       |      |
|-----------|--------|---------------|-------|------|
| 3,164,438 | 1/1965 | Thomas        | ----- | 8-46 |
| 3,203,752 | 8/1965 | Mills et al.  | ----- | 8-75 |
| 3,240,552 | 3/1966 | Joyner et al. | ----- | 8-39 |

## References Cited

## UNITED STATES PATENTS

3,148,936 9/1964 Turbak ----- 8-55

5 J. TRAVIS BROWN, *Acting Primary Examiner.*D. LEVY, *Assistant Examiner.*